

Oct. 6, 1931.

R. HERVIG

1,826,544

BLANK AND PROCESS FOR MAKING VALVE TAPPETS

Filed Jan. 11, 1926



Inventor  
Richard Hervig  
By Ellison, Mann & Co.

Attorneys

## UNITED STATES PATENT OFFICE

RICHARD HERVIG, OF DETROIT, MICHIGAN, ASSIGNOR TO RICH TOOL COMPANY, OF DETROIT, MICHIGAN, A CORPORATION OF MAINE

## BLANK AND PROCESS FOR MAKING VALVE TAPPETS

Application filed January 11, 1926. Serial No. 80,426.

Metals that can long endure in the heads of valve tappets are either excessively expensive or very difficult to machine, or both, while metals that can be readily machined, or can be purchased at reasonable cost, are not able to endure in the heads of valve tappets.

The principal object of this invention is to produce a tappet having its head and shank of different metals suited respectively to those portions and firmly united without stress or strain on the metals at, or adjacent to, the joint.

This object is attained by the structure and procedure illustrated in the accompanying drawings in which

Fig. 1 is a sectional view through a finished tappet of the preferred form;

Fig. 2 is a sectional view through a head blank for producing the tappet shown in Fig. 1; and

Fig. 3 is a sectional view through the head and stem blanks and a bottom die suitable for forging them to the form and condition indicated in Fig. 1.

The preferred form of head blank 10, illustrated in Fig. 2, may be produced by casting, by forging a ball shaped blank with suitable dies, by subjecting a bar to a Bradley hammer, or in any other way that may be selected. This blank roughly approximates the head of the finished tappet and requires no great amount of forging to give the completely finished form and secure it to the stem.

The underside of the blank, as shown in Fig. 2, is equipped with a central boss 11 surrounded by an annular flange 12, whereby an annular groove 13 is prepared for receiving the corresponding end of a tubular shank 14 in the relation illustrated in Fig. 3.

With the parts assembled as indicated in this figure, the shank is supported at proper height by a knock-out plug 15 and the head blank 10 is acted upon by a hammer or flat die to force it to fill the cavity 16 in the bottom die 17.

The upper surface of the blank 10 is provided with a disk-like recess 18 to cause the initial forging operation to affect the outer portion of the blank chiefly and cause the an-

nular flange 12 to flow well down into the cavity 16 and around the end of the shank 14. The result of this operation is illustrated in Fig. 1, where the end portion of the shank has been forged to form a flaring flange 19 above a reduction, or constriction 20, and the boss 11 and flange 12 are made to grip the flaring flange 19 and firmly secure it in what was formerly the groove 13.

Both the head and shank blanks should be heated during the forging operation so that in cooling they can shrink together and leave the metal of the two blanks in intermediate contact throughout the mating surfaces without stress or strain in either part. If, for example, the shank is forged cold, there will be some movement along the surfaces of contact as the head metal cools and shrinkage strains will remain in the head metal after cooling which, to a greater or less extent, initiates the joint.

The blanks may be heated in any suitable manner, but preferably they are brought to a forging temperature after being assembled in the die by the application of suitable electric current. One electrode may be applied to the bottom die and the other to the head blank 10. The latter can be readily arranged to move to one side when the upper die descends.

The head metal may be of any material of sufficient hardness, or capable of having sufficient hardness imparted to it. High speed tool steel or steel containing tungsten as a hardening material or wear resisting element is very suitable; cast material that is forgible when in cast form may be used; an alloy composed of sixty (60%) percent cobalt, thirty (30%) percent chromium and the remainder chiefly iron, makes a very satisfactory head. Another alloy containing sixty (60%) percent nickel, thirty (30%) percent chromium, seven (7%) percent aluminum, and the principal remainder iron, is also satisfactory.

The shank blanks may be made of a great variety of readily machined material, ordinarily .10% to .20% carbon steel, with or without three and one-half percent (3½%) nickel, is very satisfactory. This material can be readily carburized after finishing and

before forging. .50% carbon steel may be used and hardened in oil if carburizing is not resorted to to obtain suitable hardness.

I claim as my invention:

- 5 1. The process which includes forming a head blank with an annular recess on the bottom, inserting a tubular shank in the recess and forging a flange on the shank, and gripping the flange between portions of the head blank metal, the initial forging operation being directed chiefly to the marginal portion of the head blank to force the metal downwardly and inwardly against the shank.
- 10 2. The process which includes forming a head blank with a boss on the bottom surrounded by a flange, and a marginal projection on the top, resting the head blank on a tubular shank and simultaneously forging a flange on the shank and gripping the flange between the boss and the surrounding flange on the head blank, the marginal projection serving to provide extra metal in that area and to facilitate the movement of the metal in the bottom flange for the specified purpose.
- 15 3. A blank of the class described, having on the bottom a boss surrounded by a flange, and on top a marginal flange.
- 20
- 25

In testimony whereof I affix my signature.  
RICHARD HERVIG.

30

35

40

45

50

55

60

65